

## UNITED STATES PATENT OFFICE

2,080,110

## BRIDGE WIRE

Bert Brenner, Union, N. J., assignor to Sigmund Cohn, New York, N. Y.

No Drawing. Application September 17, 1936,  
Serial No. 101,269

## 3 Claims. (Cl. 75—172)

This invention relates to improvements in bridge wire for blasting cap resistance units or any resistance wire used to set off explosives, and has for its object the provision of a new alloy for such devices which is stronger and cheaper than such as have been available heretofore.

The most effective alloy for resistance units for electrically operated blasting caps has been, until now, made of twenty percent (20%) iridium and eighty percent (80%) platinum. A wire made of this alloy possesses the desirable property of resisting corrosion, is fairly strong, chemically homogeneous and constant in its electrical characteristics. Because of these desirable qualities it came to be generally used in spite of the fact that it is quite costly.

I have discovered that an alloy of rhodium, ruthenium and platinum possesses all of the desirable characteristics of the iridium-platinum alloy formerly used and that it has several important features of advantage over it. For example, a wire made of an alloy of fifteen percent (15%) rhodium, five percent (5%) ruthenium and eighty percent (80%) platinum, has about one hundred percent (100%) higher tensile strength than one made of the aforesaid iridium-platinum alloy of the same diameter. By reason of the lower specific gravity and lower specific resistance it is also possible to use a thinner wire for a given resistance and still have this wire stronger mechanically, say of fifty percent (50%) more tensile strength than said platinum-iridium wire of the same resistance.

The specific gravity and specific resistance of my new alloy are less than that of the iridium-platinum alloy, so that there is greater length in a given weight. These facts together enable the purchaser to obtain an increase of approximately thirty percent (30%) in length of wire per unit of weight at a certain resistance. This is important as it is usually sold by weight.

As the market price for rhodium and ruthenium is generally only about half that of iridium, in addition to the above advantage of greater length per unit weight there is a considerable saving in price. The intrinsic values of my alloy and twenty percent (20%) iridium-platinum are now about \$59.00 and \$72.00, respectively. This represents a saving of about eighteen percent (18%) which, added to the thirty percent (30%) saving described above and due to the more favorable specific gravity and specific resistance, makes a total saving figured on a dollar basis of forty-eight percent (48%). These prices may fluctu-

ate. They indicate, however, an approximate proportion.

|                | Price   | Pt—Ir<br>alloy |         | Pt—Rh—<br>Ru alloy |         | 5  |
|----------------|---------|----------------|---------|--------------------|---------|----|
|                |         | Percent        |         | Percent            |         |    |
| Platinum.....  | \$60.00 | 80             | \$48.00 | 80                 | \$48.00 |    |
| Iridium.....   | 120.00  | 20             | 24.00   | 15                 | 9.00    | 10 |
| Rhodium.....   | 60.00   | —              | —       | 5                  | 2.00    |    |
| Ruthenium..... | 40.00   | —              | —       | —                  | —       |    |
|                |         |                | \$72.00 |                    | \$59.00 |    |

The temperature coefficient of electrical resistance of this alloy is about forty percent (40%) lower than that of the aforesaid platinum-iridium alloy. This is an added advantage since the change in resistance is less than with the platinum-iridium alloy in the temperatures surrounding blasting operations, which may be between  $-50^{\circ}$  F. to  $+150^{\circ}$  F.

The particular alloy described is typical of a series of alloys consisting of various proportions of rhodium, ruthenium and platinum, all having similar characteristics and advantages. I have found that the practical limits within which the proportion of the three metals may be varied are:

|                |         |    |
|----------------|---------|----|
| Rhodium.....   | 2-25%   | 20 |
| Ruthenium..... | 2-15%   | 30 |
| Platinum.....  | Balance |    |

The following table is a comparison of the two alloys:

|                                                                                    | Platinum<br>20 percent<br>iridium | Platinum<br>15 Rh-5 Ru | 35 |
|------------------------------------------------------------------------------------|-----------------------------------|------------------------|----|
| Melting point $^{\circ}$ C.....                                                    | 1900                              | 1830                   |    |
| Specific gravity.....                                                              | 21.57                             | 18.7                   | 40 |
| Resistance per mil foot at $20^{\circ}$ C.....                                     | 220                               | 182                    |    |
| Temperature coefficient of resistance per $^{\circ}$ C. (0-100 $^{\circ}$ C.)..... | .0008                             | .0005                  |    |
| Ultimate tensile strength (hard) pounds per square inch.....                       | 140.500                           | 300.000                |    |
| Elongation percent (hard).....                                                     | 2.5%                              | 2.5%                   |    |
| Approximate length in feet per ounce per 100 ohms per foot at $20^{\circ}$ C.....  | 4150                              | 5600                   | 45 |

I have described my alloy as used for the resistance units or bridge wires in electrically operated blasting caps, as that is a use for which it is particularly adapted, but I desire and intend to claim it for any other use or uses to which it may be adaptable.

What I claim is:

1. An alloy for resistance units comprising rhodium, ruthenium and platinum in the propor-

tions of 2% to 25% rhodium, 2% to 15% ruthenium, and the balance platinum.

2. An alloy for resistance units comprising rhodium, ruthenium and platinum in the proportions of 15% rhodium, 5% ruthenium and 80% platinum.

3. An alloy for resistance units substantially

composed of rhodium, ruthenium and platinum in the proportions of 2% to 25% rhodium, 2% to 15% ruthenium, and 60% to 96% platinum, having the characteristics herein described, including high tensile strength and low temperature coefficient of resistance.

5

BERT BRENNER.